

[54] METHOD OF CORROSION INHIBITION IN AQUEOUS MEDIUMS

[75] Inventors: Gary E. Geiger, Philadelphia; Roger C. May, Glenside, both of Pa.

[73] Assignee: Betz Laboratories, Inc., Trevose, Pa.

[21] Appl. No.: 267,840

[22] Filed: May 28, 1981

#### Related U.S. Application Data

[63] Continuation of Ser. No. 131,593, Mar. 19, 1980, abandoned, which is a continuation-in-part of Ser. No. 27,346, Apr. 5, 1979, abandoned.

[51] Int. Cl.<sup>3</sup> C23F 11/04

[52] U.S. Cl. 422/16; 422/15; 422/17; 422/19; 252/389 R; 252/389 A

[58] Field of Search 422/7, 13, 14, 15-19; 252/389 R; 210/58, 59, 696, 698

#### References Cited

##### U.S. PATENT DOCUMENTS

- 2,872,281 2/1959 Kahler ..... 422/19  
 2,900,222 8/1959 Kahler .....  
 3,432,428 3/1969 Wirth, Jr. .....  
 3,463,730 8/1969 Booth et al. .....  
 3,532,639 10/1970 Hatch .....  
 3,663,448 5/1972 Ralston .....  
 3,766,077 10/1973 Hwa et al. .....

- 3,790,610 2/1974 Lum et al. ....  
 3,803,047 4/1974 Hwa .....  
 3,880,765 4/1975 Watson .....  
 3,885,914 5/1975 Hollingshaw et al. .... 252/180  
 3,890,228 6/1975 Hwa et al. ....  
 3,948,792 4/1976 Watsén et al. ....  
 3,965,027 6/1976 Boffardi et al. .... 252/180  
 3,992,318 11/1976 Gaupp et al. ....  
 4,018,701 4/1977 Ralston et al. .... 252/389 A  
 4,018,702 4/1977 Boffardi et al. ....  
 4,029,577 6/1977 Godlewski et al. .... 210/58  
 4,066,398 1/1978 Hwa .....  
 4,089,796 5/1978 Harris et al. ....  
 4,120,655 10/1978 Crambes et al. ....  
 4,163,733 8/1979 Buckman et al. ....  
 4,209,398 6/1980 Ti et al. ....

Primary Examiner—Ferris H. Lander

Attorney, Agent, or Firm—Alexander D. Ricci; Bruce E. Peacock

#### [57] ABSTRACT

A method for reducing corrosion of metal surfaces is disclosed according to which a specific corrosion inhibitor is utilized. The inhibitor comprises water-soluble zinc compound, water-soluble chromate compound and copolymer of acrylic acid and hydroxylated lower alkyl acrylate. Water-soluble orthophosphate can also be used.

23 Claims, 7 Drawing Figures



FIG. 1.





FIG. 2.



FIG. 3.



FIG. 4.



FIG. 5.



FIG. 6.



FIG. 7.

## METHOD OF CORROSION INHIBITION IN AQUEOUS MEDIA

This is a continuation of application Ser. No. 131,593, filed on Mar. 19, 1980, now abandoned, which, in turn, is a continuation-in-part of application Ser. No. 027,346, filed Apr. 5, 1979, abandoned.

The present invention is related to zinc-containing corrosion inhibitor treatments. The ability of zinc to inhibit the corrosion of ferrous metals is, indeed, well known. Accordingly, soluble zinc salts are vital ingredients of many corrosion treatment programs. For example, U.S. Pat. No. 4,089,796 to Harris et al discloses a corrosion inhibiting composition comprising zinc and hydrolyzed polymaleic anhydride or soluble salt thereof. Other exemplary patents disclosing such zinc-containing treatments are U.S. Pat. No. 3,432,428 to Wirth et al and U.S. Pat. No. 4,120,655 to Crambes et al.

An art-recognized major problem encountered with zinc-containing treatments, particularly in cooling water, is the uncontrolled precipitation of zinc salts; because, to be effective, the zinc must reach the surfaces to be protected in a soluble form. For example, the use of orthophosphate in combination with zinc as a cooling water treatment is well known as evidenced by U.S. Pat. No. 2,900,222 to Kahler et al. The orthophosphate can be provided as an actual addition, or as a reversion product from any one of complex inorganic phosphate, organic phosphate or organic phosphonate. When orthophosphate and zinc are both present in the water, zinc phosphate precipitation becomes a concern. Whether or not orthophosphate is present, the zinc could precipitate in other forms, for example, as zinc hydroxide or zinc silicate. The solubility of the various salts, that is, the retention of the respective salt constituents in ionic form, depends on such factors as water temperature and pH and ion concentrations. Wirth et al states that although water temperatures can vary from 32° to 200° F., lower temperatures of 32° to 80° F. are preferred because "zinc tends to remain in solution better in cooler waters." This patent further states that alkaline waters, particularly above about pH 7.5, are relatively undesirable because "the dissolved zinc tends to deposit out or drop out much more rapidly in alkaline water". Similarly, Crambes et al points out that zinc salts are unstable in neutral or alkaline water and will precipitate with phosphate. Thus, if any of these conditions are present, the aqueous medium becomes prone to zinc precipitation. Because of the formation of this zinc scale, many of the surfaces in contact with the aqueous medium will foul and the amount of effective (soluble) corrosion inhibitor present in the aqueous medium can be significantly reduced.

Although the present invention is considered to have general applicability to any aqueous system where zinc precipitation is a problem, it is particularly useful in cooling water systems. Accordingly, the invention will hereinafter be described as it relates to cooling water systems.

### DESCRIPTION OF THE INVENTION

There has existed for a long time the need for a zinc-containing corrosion inhibitor treatment which overcomes the above-noted problems, and the present invention is considered to fulfill that need.

According to the present invention, a corrosion inhibitor treatment for metal surfaces exposed to an aque-

ous medium comprises (i) water-soluble zinc compound, (ii) water-soluble chromate compound and (iii) a particular type of water-soluble polymer composed essentially of moieties derived from acrylic acid or derivatives thereof and hydroxylated lower alkyl acrylate moieties (HAA). The treatment could additionally comprise (iii) orthophosphate. It was discovered that, although the polymer demonstrated no significant activity alone as a corrosion inhibitor, when it was combined with a zinc-containing treatment the various ionic constituents of the treatment were unexpectedly retained in their soluble form and a corresponding increase in corrosion inhibiting activity was observed.

### The Polymer

The polymers according to the present invention are those effective for the purpose which contain essentially moieties derived from an acrylic acid compound (AA), i.e.,



where R is hydrogen or a lower alkyl of from 1 to 3 carbon atoms and R<sub>1</sub> = OH, NH<sub>2</sub> or OM, where M is a water-soluble cation, e.g., NH<sub>4</sub>, alkali metal (K, Na), etc; and moieties of an hydroxylated lower alkyl (C<sub>2</sub>–C<sub>6</sub>) acrylate (HAA) as represented, for example, by the formula:



where R<sub>3</sub> is H or lower alkyl of from 1 to 3 carbon atoms, and R<sub>2</sub> is a lower alkyl having from about 2 to 6 carbon atoms.

In terms of mole ratios, the polymers are considered, most broadly, to have a mole ratio of AA:HAA of from about 1:4 to 36:1. This mole ratio is preferably about 1:1 to 11:1, and most preferably about 1:1 to 5:1. The only criteria that is considered to be of importance with respect to mole ratios is that it is desirable to have a copolymer which is water-soluble. As the proportion of hydroxylated alkyl acrylate moieties increases, the solubility of the copolymer decreases. It is noted that, from an efficacy point of view, the polymers having a mole ratio of AA:HAA of 1:1 to 5:1 were considered the best.

The polymers could have a molecular weight of from about 1,000 to about 50,000 with from about 2,000 to about 6,000 being preferred.

The polymers utilized in accordance with the invention can be prepared by vinyl addition polymerization or by treatment of an acrylic acid or salt polymer. More specifically, acrylic acid or derivatives thereof or their water soluble salts, e.g., sodium, potassium, ammonium, etc. can be copolymerized with the hydroxy alkyl acrylate under standard copolymerization conditions utiliz-

ing free radical initiators such as benzoyl peroxide, azobisisobutyronitrile or redox initiators such as ferrous sulfate and ammonium persulfate. The molecular weights of the resulting copolymer can be controlled utilizing standard chain control agents such as secondary alcohols (isopropanol), mercaptans, halocarbons, etc. Copolymers falling within the scope of the invention are commercially available from, for example, National Starch Company.

The hydroxy alkyl acrylate can be prepared by the addition reaction between the acrylic acid or its derivatives or water soluble salts and the oxide of the alkyl derivative desired. For example, the preferred monomer of the present invention is the propyl derivative. Accordingly, to obtain the hydroxylated monomer, 15 acrylic acid is reacted with propylene oxide to provide the hydroxypropyl acrylate monomer.

The polymers of the invention may also be prepared by reacting a polyacrylic acid or derivatives thereof with an appropriate amount of an alkylene oxide having from 2 to 6 carbon atoms such as ethylene oxide, propylene oxide and the like. The reaction takes place at the COOH or COM group of the moieties to provide the hydroxylated alkyl acrylate moiety.

The polymer prepared either by copolymerization of 25 AA with hydroxy propyl acrylate (HPA) or reaction of AA with propylene oxide would be composed of units or moieties having the structural formulas:



where M is as earlier defined.

#### The Zinc Compounds

Illustrative water-soluble zinc compounds which are 45 considered to be suitable for use in accordance with the present invention are zinc oxide, zinc acetate, zinc chloride, zinc formate, zinc nitrate, zinc sulphate, zinc borate, etc.

#### The Orthophosphate Compounds

As already noted above, the treatment could further comprise orthophosphate. Indeed, the use of zinc and orthophosphate together as a corrosion inhibition treatment is well known. It has also already been noted that the orthophosphate could be provided as an actual addition product, e.g., sodium orthophosphate, or as a precursor compound such as complex inorganic phosphates, organic phosphates or organic phosphonates which revert to orthophosphate in the water.

Illustrative examples of orthophosphate as an actual addition are monosodium phosphate and monopotassium phosphate. Any other water-soluble orthophosphate or phosphoric acid would also be considered to be suitable.

The complex inorganic phosphates are exemplified by sodium pyrophosphate, sodium tripolyphosphate, sodium tetraphosphate, sodium septaphosphate, sodium

decaphosphate and sodium hexametaphosphate. Either the corresponding potassium or ammonium salts or the corresponding molecularly dehydrated phosphoric acids such as metaphosphoric acid or pyrophosphoric acid are considered to be suitable.

The organic phosphonates are exemplified by amino-trimethylene phosphonic acid, hydroxyethylidene di-phosphonic acid and the water-soluble salts thereof.

Organic phosphates are exemplified in U.S. Pat. No. 3,510,436.

#### The Chromate Compounds

As disclosed in U.S. Pat. No. 2,900,222 to Kahler et al, the chromate compounds would include alkali metals or any water-soluble compound that contains hexavalent chromate and provides chromate radical in water solutions. Illustrative water-soluble chromate compounds are sodium chromate dihydrate, sodium chromate anhydrous, sodium chromate tetrahydrate, sodium chromate hexahydrate, sodium chromate decahydrate, potassium dichromate, potassium chromate, ammonium dichromate and chromic acid.

The amount of each constituent added to the cooling water will, of course, be an effective amount for the purpose and will depend on such factors as the nature and severity of the corrosion problem being treated, the temperature and pH of the cooling water and the type and amount of precipitation-prone ions present in the water.

30 In terms of active zinc ion, as little as about 0.5 parts of zinc per million parts (ppm) of cooling water are believed to be effective in certain instances, with about 2 ppm being preferred. Based on economic considerations, the amount of zinc ion added could be as high as about 25 ppm, with about 10 ppm representing the preferred maximum.

35 In terms of active polymer, as little as about 0.5 ppm polymer is considered to be effective, while about 2 ppm is the preferred minimum. Based on economic considerations, the polymer could be fed in amounts as high as about 200 ppm, with about 50 ppm representing the preferred maximum.

40 In terms of active product added, the orthophosphate or precursor compound thereof could be fed in an amount as low as about 1 ppm, with about 2 ppm representing the preferred minimum. Based on economic considerations, the maximum amount is considered to be about 200 ppm. However, about 50 ppm is considered to be the preferred maximum.

45 In terms of active chromate compound added, as little as about 1 ppm is considered to be effective. The upper limit would depend on such factors as cost and toxicity and could be as high as about 150 ppm. The preferred upper limit is about 50 ppm.

50 Methods for feeding corrosion inhibitors to cooling water are well known in the art such that details thereof are not considered necessary. However, due to rather severe stability problems experienced when the polymer was stored at high concentrations with remaining components, a two or three-barrel treatment is recommended.

55 The cooling water to be treated preferably will have a pH of about 6.5 to about 9.5. Since zinc precipitation problems most commonly occur at pH's above about 7.5, the most preferred pH range is from about 7.5 to about 9.5. Kahler et al, U.S. Pat. No. 2,900,222, points out that the use of chromate in cooling water treatments

permits the treatment of cooling water at lower pH's e.g., pH 5.7.

### EXAMPLES

#### Illustration of Zinc Precipitation Problem

5

##### Example 1

As noted above, an art-recognized major problem encountered with zinc-containing treatments, particularly in cooling water, is the uncontrolled precipitation of zinc salts from the water. Even in the absence of orthophosphate in the water, the zinc can form precipitates such as zinc hydroxide.

This point is illustrated by the zinc-solubility results of several tests conducted in water containing no orthophosphate. The tests were conducted, inter alia, to determine the solubility of zinc in the test water as a function of pH.

The following aqueous test solutions were first prepared:

Solution A: 1,000 ppm  $Zn^{++}$  obtained from 0.27 gram  $ZnSO_4 \cdot H_2O$ /100 ml

SCW<sub>7</sub>:

170 ppm Ca as  $CaCO_3$

110 ppm Mg as  $CaCO_3$

15 ppm  $SiO_2$

The tests were conducted using the following procedure:

1. Prepare SCW<sub>7</sub> (detailed in Example 5 below) and adjust its pH to 4 with concentrated HCl.

2. To 2,000 ml of the above solution, add the required amount of Solution A with stirring.

3. Add 100 ml of the solution from step 2 to a bottle and agitate.

4. Slowly adjust the pH to the desired value with dilute NaOH solution and record pH.

5. Place the samples in an oven at the required temperature for 24 hours, after which time, filter through a 0.2 micron millipore filter.

6. Analyze the filtrate for soluble zinc and record final pH.

The results of these tests are reported below in Tables 1 and 2 in terms of soluble zinc (ppm) remaining after 24 hours at various final pH values.

TABLE 1

| ZINC PRECIPITATION AS FUNCTION OF pH |                                   |  |
|--------------------------------------|-----------------------------------|--|
| Conditions:                          | Initial Zinc = 2 ppm as $Zn^{++}$ |  |
| T                                    | = 120° F.                         |  |
| Time                                 | = 24 hours                        |  |
| pH                                   | soluble zinc (ppm)                |  |
| 7.62                                 | 0.8                               |  |
| 7.70                                 | 0.5                               |  |
| 7.92                                 | 0.5                               |  |
| 8.12                                 | 0.2                               |  |
| 8.21                                 | 0.1                               |  |
| 8.35                                 | 0.2                               |  |
| 8.42                                 | 0.1                               |  |
| 8.76                                 | 0.0                               |  |

TABLE 2

| ZINC PRECIPITATION AS FUNCTION OF pH |                                    |  |
|--------------------------------------|------------------------------------|--|
| Conditions:                          | Initial Zinc = 10 ppm as $Zn^{++}$ |  |
| T                                    | = 120° F.                          |  |
| Time                                 | = 24 hours                         |  |
| pH                                   | soluble zinc (ppm)                 |  |
| 7.15                                 | 8.2                                |  |
| 7.25                                 | 7.8                                |  |
| 7.36                                 | 8.2                                |  |
| 7.46                                 | 8.0                                |  |

TABLE 2-continued

| ZINC PRECIPITATION AS FUNCTION OF pH |                                    |  |
|--------------------------------------|------------------------------------|--|
| Conditions:                          | Initial Zinc = 10 ppm as $Zn^{++}$ |  |
| T                                    | = 120° F.                          |  |
| Time                                 | = 24 hours                         |  |
| pH                                   | soluble zinc (ppm)                 |  |
| 7.50                                 | 7.8                                |  |
| 7.56                                 | 5.4                                |  |
| 7.67                                 | 1.8                                |  |
| 7.70                                 | 1.6                                |  |
| 8.05                                 | 0.4                                |  |
| 8.10                                 | 0.2                                |  |
| 8.22                                 | 0.4                                |  |
| 8.65                                 | 0.2                                |  |
| 9.06                                 | 0.0                                |  |

EXAMPLE 2

The problem of zinc precipitation in cooling water is further illustrated by the zinc-solubility results of additional tests similar to those in Example 1, but conducted in water containing both zinc ions and orthophosphate ions.

The following aqueous test solutions were first prepared:

Solution A: 1,000 ppm  $PO_4^{3-}$ , obtained from 0.400 gram  $Na_3PO_4 \cdot 12H_2O$ /100 ml

Solution B: 1,000 ppm  $Zn^{++}$ , obtained from 0.27 gram  $ZnSO_4 \cdot H_2O$ /100 ml

SCW<sub>7</sub>: Same as Example 1

The following procedure was used:

1. Prepare SCW<sub>7</sub> and adjust its pH to 4 with HCl solution.

2. To 2,000 ml of the above solution, add the appropriate amount of Solution A, followed by the appropriate amount of Solution B with agitation.

3. Add 100 ml of the solution from step 2 to a bottle and adjust the pH to 7.5 with dilute NaOH with agitation.

4. Place the samples in an oven for 24 hours at the appropriate temperature.

5. After the 24 hour period, filter the solution through a 0.2 micron millipore filter.

6. Analyze the filtrate for  $Zn^{++}$  and  $PO_4^{3-}$ .

The results of these tests are reported below in Tables 3 and 4 in terms of ppm soluble zinc and ppm soluble phosphate remaining after 24 hours at various final pH values.

TABLE 3

| ZINC PRECIPITATION AS FUNCTION OF pH |                                   |  |
|--------------------------------------|-----------------------------------|--|
| Conditions:                          | Initial Zinc = 5 ppm as $Zn^{++}$ |  |
| Initial $PO_4^{3-}$                  | = 10 ppm                          |  |
| T                                    | = 120° F.                         |  |
| Time                                 | = 24 hours                        |  |
| pH                                   | soluble zinc (ppm)                |  |
| 7.0                                  | 3                                 |  |
| 7.5                                  | 0.5                               |  |
| 8.0                                  | 0.1                               |  |
| 8.5                                  | 0.1                               |  |
| 9.0                                  | 0.1                               |  |
| pH                                   | soluble $PO_4^{3-}$ (ppm)         |  |
| 7.0                                  | 6                                 |  |
| 7.5                                  | 5                                 |  |
| 8.0                                  | 3.7                               |  |
| 8.5                                  | 2.4                               |  |
| 9.0                                  | 1.2                               |  |

TABLE 4

| ZINC PRECIPITATION AS FUNCTION OF pH |                                    |                                 |
|--------------------------------------|------------------------------------|---------------------------------|
| Conditions:                          | Initial Zinc = 10 ppm as $Zn^{++}$ | Initial $\text{o-PO}_4$ = 5 ppm |
| pH                                   | zinc (ppm)                         | $\text{PO}_4$ (ppm)             |
| 7.5                                  | 3.3                                | 0.8                             |
| 8.0                                  | 0.2                                | 0.7                             |
| 9.0                                  | 0.1                                | 0.1                             |

## EFFICACY IN RETAINING SOLUBLE ZINC-CONTAINING TREATMENTS

## Example 3

A series of tests were conducted to determine the efficacy of various materials in retaining zinc-containing corrosion inhibition treatments in a soluble form. After all, the corrosion inhibition efficacy of such treatments will, for the most part, depend on the constituents remaining soluble.

The test water contained both zinc and orthophosphate ions, and the test procedures were the same as in Example 2 but for a few different steps as follows:

1. Solution C, comprising 1,000 ppm of active treatment, was also used.

3. Add 100 ml of solution from step 2 to a bottle, add the appropriate quantity of treatment solution (1 ml = 10 ppm), and adjust pH to appropriate value with dilute NaOH with agitation.

10 The results of the tests were calculated in terms of % increase in retention of soluble zinc ions and soluble phosphate ions vs. an untreated solution using the following equation:

15

$$\% \text{ Retention} = \frac{100 \times \text{Sol. PO}_4 \text{ at } T = 24 \text{ hrs} - \text{Sol. PO}_4 \text{ in control at } T = 24 \text{ hrs.}}{\text{Sol. PO}_4 \text{ in control at } T = 0 \text{ hrs} - \text{Sol. PO}_4 \text{ in control at } T = 24 \text{ hrs.}}$$

20 where Sol.  $\text{PO}_4$  = soluble  $\text{PO}_4$  in ppm. Of course, a similar equation was used for zinc calculations.

The results of these tests are reported below in Tables 5 and 6. In addition to testing various AA/HPA copolymers in accordance with the present invention, various commercial polyacrylic acids (PAA) were also tested.

TABLE 5

## ZINC AND PHOSPHATE RETENTION

Conditions: Initial Zinc = 10 ppm as  $Zn^{++}$   
Initial  $\text{o-PO}_4$  = 5 ppm  
T = 120° F.  
Time = 24 hours

| Treatment      | Mole Ratio AA:HPA | Molecular Weight | Water pH | Dosage (ppm actives) | Soluble Zinc Retained (ppm) | Soluble $\text{PO}_4$ Retained (ppm) | % Increase in Zinc Retention (vs. Control) | % Increase in $\text{PO}_4$ Retention (vs. Control) |
|----------------|-------------------|------------------|----------|----------------------|-----------------------------|--------------------------------------|--------------------------------------------|-----------------------------------------------------|
| None           | —                 | —                | 7.5      | —                    | 3.3                         | 0.8                                  | —                                          | —                                                   |
| PAA-Commercial | —                 | 5,000            | 7.5      | 5                    | 2.3                         | 0.8                                  | -15                                        | 0                                                   |
| PAA-Commercial | —                 | 5,000            | 7.5      | 10                   | 2.3                         | 1.0                                  | -15                                        | 5                                                   |
| PAA-Commercial | —                 | 5,000            | 7.5      | 20                   | 2.4                         | 1.2                                  | -13                                        | 10                                                  |
| PAA-Commercial | —                 | 90,000           | 7.5      | 5                    | 2.2                         | 0.7                                  | -16                                        | 0                                                   |
| PAA-Commercial | —                 | 90,000           | 7.5      | 10                   | 2.5                         | 1.0                                  | -12                                        | 5                                                   |
| PAA-Commercial | —                 | 90,000           | 7.5      | 20                   | 1.9                         | 1.4                                  | -21                                        | 14                                                  |
| PAA-Commercial | —                 | <1,000           | 7.5      | 5                    | 2.9                         | 0.9                                  | -6                                         | 2                                                   |
| PAA-Commercial | —                 | <1,000           | 7.5      | 10                   | 3.4                         | 1.4                                  | 1                                          | 14                                                  |
| PAA-Commercial | —                 | <1,000           | 7.5      | 20                   | 3.0                         | 1.2                                  | -4                                         | 10                                                  |
| AA/HPA 1:8:1   | 6,000             | 7.5              | 2.5      | 3.7                  | 1.2                         | 6                                    | 10                                         |                                                     |
| AA/HPA 1:8:1   | 6,000             | 7.5              | 5        | 8.6                  | 4.2                         | 79                                   | 81                                         |                                                     |
| AA/HPA 3:1     | 6,000             | 7.5              | 2.5      | 1.3                  | 1                           | -30                                  | 5                                          |                                                     |
| AA/HPA 3:1     | 6,000             | 7.5              | 5        | 8.6                  | 4.4                         | 79                                   | 86                                         |                                                     |
| AA/HPA 9:9:1   | 1K-2K*            | 7.5              | 5        | 6.8                  | 4.7                         | 52                                   | 93                                         |                                                     |
| AA/HPA 9:9:1   | 1K-2K             | 7.5              | 10       | 8.6                  | 5.1                         | 79                                   | 102                                        |                                                     |
| AA/HPA 9:9:1   | 6-10K             | 7.5              | 5        | 8.8                  | 4.7                         | 82                                   | 93                                         |                                                     |
| AA/HPA 9:9:1   | 6K-10K            | 7.5              | 10       | 7.2                  | 4.8                         | 58                                   | 95                                         |                                                     |
| AA/HPA 19:8:1  | 2K-6K             | 7.5              | 5        | 5.4                  | 2.8                         | 31                                   | 48                                         |                                                     |
| AA/HPA 19:8:1  | 2K-6K             | 7.5              | 10       | 5.6                  | 3.2                         | 34                                   | 57                                         |                                                     |
| AA/HPA 36:1    | 2K-6K             | 7.5              | 5        | 6.8                  | 4.3                         | 52                                   | 83                                         |                                                     |
| AA/HPA 36:1    | 2K-6K             | 7.5              | 10       | 8.8                  | 4.8                         | 82                                   | 95                                         |                                                     |

\*K = 1,000

TABLE 6

| ZINC AND PHOSPHATE RETENTION                                                                                          |                   |                          |             |                            |                                        |                                                   |                                                       |                                                                  |
|-----------------------------------------------------------------------------------------------------------------------|-------------------|--------------------------|-------------|----------------------------|----------------------------------------|---------------------------------------------------|-------------------------------------------------------|------------------------------------------------------------------|
| Conditions: Initial Zinc = 5 ppm as $Zn^{++}$<br>Initial o-PO <sub>4</sub> = 10 ppm<br>T = 120° F.<br>Time = 24 hours |                   |                          |             |                            |                                        |                                                   |                                                       |                                                                  |
| Treatment                                                                                                             | Mole Ratio AA:HPA | Mole-<br>cular<br>Weight | Water<br>pH | Dosage<br>(ppm<br>actives) | Soluble<br>Zinc Re-<br>tained<br>(ppm) | Soluble<br>PO <sub>4</sub> Re-<br>tained<br>(ppm) | % Increase<br>in Zinc Re-<br>tention (vs.<br>Control) | % Increase<br>in PO <sub>4</sub> Re-<br>tention (vs.<br>Control) |
| None                                                                                                                  | —                 | —                        | 7.0         | —                          | 3                                      | 6                                                 | —                                                     | —                                                                |
| AA/HPA                                                                                                                | 1.8:1             | 6,000                    | 7.0         | 2.5                        | 4.6                                    | 9.2                                               | 80                                                    | 80                                                               |
| "                                                                                                                     | 1.8:1             | 6,000                    | 7.0         | 5                          | 4.9                                    | 9.5                                               | 95                                                    | 87                                                               |
| "                                                                                                                     | 3:1               | 6,000                    | 7.0         | 2.5                        | 4.2                                    | 8.9                                               | 60                                                    | 72                                                               |
| "                                                                                                                     | 3:1               | 6,000                    | 7.0         | 5                          | 5                                      | 9.4                                               | 100                                                   | 85                                                               |
| "                                                                                                                     | 9.9:1             | 1K-2K*                   | 7.0         | 2.5                        | 4.9                                    | 9.3                                               | 95                                                    | 82                                                               |
| "                                                                                                                     | 9.9:1             | 1K-2K                    | 7.0         | 5                          | 5.0                                    | 9.4                                               | 100                                                   | 85                                                               |
| "                                                                                                                     | 9.9:1             | 6K-10K                   | 7.0         | 2.5                        | 3.2                                    | 6.8                                               | 10                                                    | 20                                                               |
| "                                                                                                                     | 9.9:1             | 6K-10K                   | 7.0         | 5                          | 5.0                                    | 9.3                                               | 100                                                   | 82                                                               |
| "                                                                                                                     | 19.8:1            | 2K-6K                    | 7.0         | 2.5                        | 4.3                                    | 8.3                                               | 65                                                    | 57                                                               |
| "                                                                                                                     | 19.8:1            | 2K-6K                    | 7.0         | 5                          | 4.7                                    | 8.9                                               | 85                                                    | 72                                                               |
| "                                                                                                                     | 36:1              | 2K-6K                    | 7.0         | 2.5                        | 4.3                                    | 8.5                                               | 65                                                    | 62                                                               |
| "                                                                                                                     | 36:1              | 2K-6K                    | 7.0         | 5                          | 4.4                                    | 8.5                                               | 70                                                    | 62                                                               |
| None                                                                                                                  | —                 | —                        | 8.0         | —                          | 0.1                                    | 3.7                                               | —                                                     | —                                                                |
| AA/HPA                                                                                                                | 1.8:1             | 6,000                    | 8.0         | 2.5                        | 1.8                                    | 5.7                                               | 35                                                    | 32                                                               |
| "                                                                                                                     | 1.8:1             | 6,000                    | 8.0         | 5                          | 3.8                                    | 8.8                                               | 75                                                    | 81                                                               |
| "                                                                                                                     | 3:1               | 6,000                    | 8.0         | 10                         | 3.8                                    | 8.8                                               | 75                                                    | 81                                                               |
| "                                                                                                                     | 9.9:1             | 1K-2K                    | 8.0         | 10                         | 3.8                                    | 9.1                                               | 75                                                    | 86                                                               |
| "                                                                                                                     | 19.8:1            | 1K-2K                    | 8.0         | 10                         | 3.7                                    | 9.1                                               | 73                                                    | 86                                                               |
| "                                                                                                                     | 36:1              | 1K-2K                    | 8.0         | 10                         | 3.9                                    | 9.1                                               | 77                                                    | 86                                                               |
| None                                                                                                                  | —                 | —                        | 9.0         | —                          | 0.1                                    | 1.2                                               | —                                                     | —                                                                |
| AA/HPA                                                                                                                | 1.8:1             | 6,000                    | 9.0         | 30                         | 4.5                                    | 8.4                                               | 90                                                    | 82                                                               |
| "                                                                                                                     | 1.8:1             | 6,000                    | 9.0         | 20                         | 4.5                                    | 8.4                                               | 90                                                    | 82                                                               |
| "                                                                                                                     | 3:1               | 6,000                    | 9.0         | 30                         | 4.6                                    | 8.5                                               | 92                                                    | 83                                                               |
| "                                                                                                                     | 3:1               | 6,000                    | 9.0         | 20                         | 4.7                                    | 8.7                                               | 94                                                    | 85                                                               |
| "                                                                                                                     | 9.9:1             | 1K-2K                    | 9.0         | 15                         | 3.5                                    | 7.6                                               | 69                                                    | 73                                                               |
| "                                                                                                                     | 9.9:1             | 1K-2K                    | 9.0         | 20                         | 4.4                                    | 7.4                                               | 88                                                    | 70                                                               |
| "                                                                                                                     | 9.9:1             | 6K-10K                   | 9.0         | 30                         | 3.0                                    | 6.5                                               | 59                                                    | 58                                                               |
| "                                                                                                                     | 9.9:1             | 6K-10K                   | 9.0         | 20                         | 4.3                                    | 8.4                                               | 86                                                    | 82                                                               |
| "                                                                                                                     | 19.8:1            | 2K-6K                    | 9.0         | 20                         | 2.4                                    | 6.7                                               | 47                                                    | 62                                                               |
| "                                                                                                                     | 36:1              | 2K-6K                    | 9.0         | 30                         | 4.1                                    | 7.9                                               | 82                                                    | 76                                                               |
| "                                                                                                                     | 36:1              | 2K-6K                    | 9.0         | 15                         | 2.9                                    | 6.7                                               | 57                                                    | 62                                                               |
| "                                                                                                                     | 36:1              | 2K-6K                    | 9.0         | 20                         | 3.9                                    | 7.4                                               | 77                                                    | 70                                                               |

\*K = 1,000

## EXAMPLE 4

A further series of tests were conducted to demonstrate the efficacy of various AA/HPA polymers in retaining soluble zinc in an aqueous medium. The tests were the same as those of Example 3 except for the absence of orthophosphate from the test solutions.

The results of these tests are reported below in Tables 7-13 in terms of ppm soluble zinc retained in solution. For purposes of comparison with untreated test solution, Table 7 should be compared with the results of Table 1 and Tables 8-13 should be compared with the results of Table 2.

Visual comparisons of Table 7 with Table 1 and Tables 8-13 with Table 2 are provided in the accompanying drawing.

In FIG. 1 are presented a series of graphs which contain comparisons of Table 7 with Table 1 in terms of soluble zinc remaining in solution after 24 hours vs. pH of the test water. As can be seen from the figure, the lowermost graph represents a no treatment test wherein the zinc readily precipitates. In comparison, the higher graphs represent various test solutions to which have been added the noted AA/HPA polymers. The polymers were all considered to be efficacious in retaining soluble zinc in solution.

Remaining FIGS. 2-7 provide visual comparisons of respective ones of Tables 8-13 with Table 2. FIG. 2 compares Table 8, FIG. 3 compares Table 9, FIG. 4 compares Table 10, FIG. 5 compares Table 11, FIG. 6

40 compares Table 12, and FIG. 7 compares Table 13, all with Table 2 in terms of plots of soluble zinc remaining in solution after 24 hours vs. pH at various indicated treatment levels. The line marked "No Treatment" in each figure represents the results of Table 2.

45

TABLE 7

| ZINC RETAINED AS COMPARED TO TABLE 1                                                                                            |                  |          |                             |  |
|---------------------------------------------------------------------------------------------------------------------------------|------------------|----------|-----------------------------|--|
| Conditions: Initial Zinc = 2 ppm as $Zn^{++}$<br>T = 120° F.<br>Time = 24 hours<br>Treatment = AA/HPA<br>Dosage = 5 ppm actives |                  |          |                             |  |
| Mole Ratio AA:HPA                                                                                                               | Molecular Weight | Water pH | Soluble Zinc Retained (ppm) |  |
| 1.8:1                                                                                                                           | 6,000            | 8.27     | 1.8                         |  |
| "                                                                                                                               | "                | 8.42     | 1.7                         |  |
| "                                                                                                                               | "                | 8.78     | 1.8                         |  |
| "                                                                                                                               | "                | 8.86     | 1.7                         |  |
| "                                                                                                                               | "                | 9.10     | 0.9                         |  |
| 9.9:1                                                                                                                           | 6,000-10,000     | 7.59     | 1.7                         |  |
| "                                                                                                                               | "                | 7.85     | 1.7                         |  |
| "                                                                                                                               | "                | 7.95     | 1.7                         |  |
| "                                                                                                                               | "                | 8.00     | 1.8                         |  |
| "                                                                                                                               | "                | 8.45     | 1.6                         |  |
| "                                                                                                                               | "                | 8.72     | 1.6                         |  |
| "                                                                                                                               | "                | 8.94     | 1.5                         |  |
| 3:1                                                                                                                             | 6,000            | 7.50     | 1.8                         |  |
| "                                                                                                                               | "                | 7.85     | 1.8                         |  |
| "                                                                                                                               | "                | 8.21     | 1.9                         |  |
| "                                                                                                                               | "                | 8.54     | 1.8                         |  |
| "                                                                                                                               | "                | 8.67     | 1.6                         |  |
| "                                                                                                                               | "                | 8.94     | 1.5                         |  |
|                                                                                                                                 | "                | 9.06     | 1.2                         |  |

TABLE 7-continued

| ZINC RETAINED AS COMPARED TO TABLE 1 |                                                                                                                            |                   |                  |          |                             |
|--------------------------------------|----------------------------------------------------------------------------------------------------------------------------|-------------------|------------------|----------|-----------------------------|
| Conditions:                          | Initial Zinc = 2 ppm as Zn <sup>++</sup><br>T = 120° F.<br>Time = 24 hours<br>Treatment = AA/HPA<br>Dosage = 5 ppm actives | Mole Ratio AA:HPA | Molecular Weight | Water pH | Soluble Zinc Retained (ppm) |
|                                      | 9.9:1                                                                                                                      | 1,000-2,000       | 7.68             | 1.9      |                             |
|                                      | "                                                                                                                          | "                 | 8.06             | 1.8      |                             |
|                                      | "                                                                                                                          | "                 | 8.21             | 1.7      |                             |
|                                      | "                                                                                                                          | "                 | 8.38             | 1.8      |                             |
|                                      | "                                                                                                                          | "                 | 8.51             | 1.5      |                             |
|                                      | "                                                                                                                          | "                 | 8.88             | 1.7      |                             |
|                                      | 19.8:1                                                                                                                     | 2,000-6,000       | 7.79             | 1.7      |                             |
|                                      | "                                                                                                                          | "                 | 7.92             | 1.8      |                             |
|                                      | "                                                                                                                          | "                 | 8.25             | 1.4      |                             |
|                                      | "                                                                                                                          | "                 | 8.50             | 1.4      |                             |
|                                      | "                                                                                                                          | "                 | 8.67             | 1.1      |                             |
|                                      | "                                                                                                                          | "                 | 8.92             | 0.7      |                             |
|                                      | 36:1                                                                                                                       | 2,000-6,000       | 7.84             | 1.7      |                             |
|                                      | "                                                                                                                          | "                 | 8.05             | 1.8      |                             |
|                                      | "                                                                                                                          | "                 | 8.65             | 1.7      |                             |
|                                      | "                                                                                                                          | "                 | 8.88             | 1.6      |                             |
|                                      | "                                                                                                                          | "                 | 8.95             | 1.6      |                             |

TABLE 9-continued

| ZINC RETAINED AS COMPARED TO TABLE 2 |                                                                                                                                                         |          |                                |                             |
|--------------------------------------|---------------------------------------------------------------------------------------------------------------------------------------------------------|----------|--------------------------------|-----------------------------|
| Conditions:                          | Initial Zinc = 10 ppm as Zn <sup>++</sup><br>T = 120° F.<br>Time = 24 hours<br>Treatment = AA/HPA, Mole Ratio AA:HPA = 3:1,<br>Molecular Weight = 6,000 | Water pH | Treatment Dosage (ppm actives) | Soluble Zinc Retained (ppm) |
|                                      | 5                                                                                                                                                       | 8.20     | 5                              | 0.8                         |
|                                      | "                                                                                                                                                       | 8.37     | 5                              | 2.0                         |
|                                      | "                                                                                                                                                       | 8.45     | 5                              | 0.8                         |
|                                      | "                                                                                                                                                       | 8.55     | 5                              | 0.0                         |
|                                      | "                                                                                                                                                       | 7.62     | 10                             | 7.8                         |
|                                      | 10                                                                                                                                                      | 7.90     | 10                             | 7.6                         |
|                                      | "                                                                                                                                                       | 8.00     | 10                             | 8.0                         |
|                                      | "                                                                                                                                                       | 8.29     | 10                             | 7.0                         |
|                                      | "                                                                                                                                                       | 8.34     | 10                             | 8.4                         |
|                                      | "                                                                                                                                                       | 8.41     | 10                             | 7.4                         |
|                                      | "                                                                                                                                                       | 8.56     | 10                             | 7.2                         |
|                                      | 15                                                                                                                                                      | 8.60     | 10                             | 8.4                         |
|                                      | "                                                                                                                                                       | 8.97     | 10                             | 6.6                         |
|                                      | "                                                                                                                                                       | 9.14     | 10                             | 7.0                         |
|                                      | "                                                                                                                                                       | 9.30     | 10                             | 4.8                         |
|                                      | "                                                                                                                                                       | 8.58     | 20                             | 9.0                         |
|                                      | "                                                                                                                                                       | 8.80     | 20                             | 9.4                         |
|                                      | "                                                                                                                                                       | 9.31     | 20                             | 8.8                         |

TABLE 8

| ZINC RETAINED AS COMPARED TO TABLE 2 |                                                                                                                                                           |          |                                |                             |
|--------------------------------------|-----------------------------------------------------------------------------------------------------------------------------------------------------------|----------|--------------------------------|-----------------------------|
| Conditions:                          | Initial Zinc = 10 ppm as Zn <sup>++</sup><br>T = 120° F.<br>Time = 24 hours<br>Treatment = AA/HPA, Mole Ratio AA:HPA = 1.8:1,<br>Molecular Weight = 6,000 | Water pH | Treatment Dosage (ppm actives) | Soluble Zinc Retained (ppm) |
|                                      | 7.50                                                                                                                                                      | 5        | 8.6                            |                             |
|                                      | 7.60                                                                                                                                                      | 5        | 10.0                           |                             |
|                                      | 7.75                                                                                                                                                      | 5        | 5.4                            |                             |
|                                      | 7.79                                                                                                                                                      | 5        | 6.6                            |                             |
|                                      | 7.92                                                                                                                                                      | 5        | 5.0                            |                             |
|                                      | 7.96                                                                                                                                                      | 5        | 4.4                            |                             |
|                                      | 8.26                                                                                                                                                      | 5        | 0.2                            |                             |
|                                      | 8.30                                                                                                                                                      | 5        | 0.6                            |                             |
|                                      | 8.42                                                                                                                                                      | 5        | 0.4                            |                             |
|                                      | 8.48                                                                                                                                                      | 5        | 1.6                            |                             |
|                                      | 8.60                                                                                                                                                      | 5        | 0.8                            |                             |
|                                      | 7.61                                                                                                                                                      | 10       | 8.0                            |                             |
|                                      | 7.70                                                                                                                                                      | 10       | 8.4                            |                             |
|                                      | 7.90                                                                                                                                                      | 10       | 8.0                            |                             |
|                                      | 8.00                                                                                                                                                      | 10       | 8.2                            |                             |
|                                      | 8.27                                                                                                                                                      | 10       | 8.4                            |                             |
|                                      | 8.75                                                                                                                                                      | 10       | 8.0                            |                             |
|                                      | 8.90                                                                                                                                                      | 10       | 8.6                            |                             |
|                                      | 9.02                                                                                                                                                      | 10       | 7.4                            |                             |
|                                      | 9.18                                                                                                                                                      | 10       | 6.8                            |                             |
|                                      | 9.23                                                                                                                                                      | 10       | 3.4                            |                             |
|                                      | 8.82                                                                                                                                                      | 20       | 9.4                            |                             |
|                                      | 8.88                                                                                                                                                      | 20       | 9.8                            |                             |
|                                      | 9.13                                                                                                                                                      | 20       | 10.0                           |                             |

TABLE 10

| ZINC RETAINED AS COMPARED TO TABLE 2 |                                                                                                                                                                 |          |                                |                             |
|--------------------------------------|-----------------------------------------------------------------------------------------------------------------------------------------------------------------|----------|--------------------------------|-----------------------------|
| Conditions:                          | Initial Zinc = 10 ppm as Zn <sup>++</sup><br>T = 120° F.<br>Time = 24 hours<br>Treatment = AA/HPA, Mole Ratio AA:HPA = 9.9:1,<br>Molecular Weight = 1,000-2,000 | Water pH | Treatment Dosage (ppm actives) | Soluble Zinc Retained (ppm) |
|                                      | 30                                                                                                                                                              | 7.60     | 5                              | 8.6                         |
|                                      | "                                                                                                                                                               | 7.72     | 5                              | 8.0                         |
|                                      | "                                                                                                                                                               | 7.80     | 5                              | 6.6                         |
|                                      | "                                                                                                                                                               | 7.93     | 5                              | 5.0                         |
|                                      | "                                                                                                                                                               | 8.04     | 5                              | 3.2                         |
|                                      | 35                                                                                                                                                              | 8.27     | 5                              | 1.2                         |
|                                      | "                                                                                                                                                               | 8.35     | 5                              | 1.0                         |
|                                      | "                                                                                                                                                               | 7.53     | 10                             | 9.0                         |
|                                      | "                                                                                                                                                               | 7.75     | 10                             | 10.0                        |
|                                      | "                                                                                                                                                               | 7.97     | 10                             | 10.0                        |
|                                      | "                                                                                                                                                               | 8.15     | 10                             | 9.4                         |
|                                      | "                                                                                                                                                               | 8.30     | 10                             | 6.6                         |
|                                      | "                                                                                                                                                               | 8.48     | 10                             | 8.4                         |
|                                      | "                                                                                                                                                               | 8.65     | 10                             | 6.8                         |
|                                      | "                                                                                                                                                               | 8.72     | 10                             | 5.6                         |
|                                      | "                                                                                                                                                               | 8.92     | 10                             | 6.0                         |
|                                      | "                                                                                                                                                               | 9.10     | 10                             | 5.0                         |
|                                      | 40                                                                                                                                                              | 9.25     | 10                             | 4.4                         |
|                                      | "                                                                                                                                                               | 8.65     | 20                             | 7.6                         |
|                                      | "                                                                                                                                                               | 8.90     | 20                             | 7.2                         |
|                                      | "                                                                                                                                                               | 9.10     | 20                             | 7.6                         |
|                                      | 45                                                                                                                                                              | 9.30     | 20                             | 3.2                         |
|                                      | "                                                                                                                                                               | 7.60     | 5                              | 8.6                         |
|                                      | "                                                                                                                                                               | 7.72     | 5                              | 8.0                         |
|                                      | "                                                                                                                                                               | 7.80     | 5                              | 6.6                         |
|                                      | "                                                                                                                                                               | 7.93     | 5                              | 5.0                         |
|                                      | "                                                                                                                                                               | 8.04     | 5                              | 3.2                         |
|                                      | 50                                                                                                                                                              | 8.27     | 5                              | 1.2                         |
|                                      | "                                                                                                                                                               | 8.35     | 5                              | 1.0                         |
|                                      | "                                                                                                                                                               | 7.53     | 10                             | 9.0                         |
|                                      | "                                                                                                                                                               | 7.75     | 10                             | 10.0                        |
|                                      | "                                                                                                                                                               | 7.97     | 10                             | 10.0                        |
|                                      | "                                                                                                                                                               | 8.15     | 10                             | 9.4                         |
|                                      | "                                                                                                                                                               | 8.30     | 10                             | 6.6                         |
|                                      | "                                                                                                                                                               | 8.48     | 10                             | 8.4                         |
|                                      | "                                                                                                                                                               | 8.65     | 10                             | 6.8                         |
|                                      | "                                                                                                                                                               | 8.72     | 10                             | 5.6                         |
|                                      | "                                                                                                                                                               | 8.92     | 10                             | 6.0                         |
|                                      | "                                                                                                                                                               | 9.10     | 10                             | 5.0                         |
|                                      | "                                                                                                                                                               | 9.25     | 10                             | 4.4                         |
|                                      | "                                                                                                                                                               | 8.65     | 20                             | 7.6                         |
|                                      | "                                                                                                                                                               | 8.90     | 20                             | 7.2                         |
|                                      | "                                                                                                                                                               | 9.10     | 20                             | 7.6                         |
|                                      | "                                                                                                                                                               | 9.30     | 20                             | 3.2                         |

TABLE 11

| ZINC RETAINED AS COMPARED TO TABLE 2 |                                                                                                                                                                  |          |                                |                             |
|--------------------------------------|------------------------------------------------------------------------------------------------------------------------------------------------------------------|----------|--------------------------------|-----------------------------|
| Conditions:                          | Initial Zinc = 10 ppm as Zn <sup>++</sup><br>T = 120° F.<br>Time = 24 hours<br>Treatment = AA/HPA, Mole Ratio AA:HPA = 9.9:1,<br>Molecular Weight = 6,000-10,000 | Water pH | Treatment Dosage (ppm actives) | Soluble Zinc Retained (ppm) |
|                                      | 60                                                                                                                                                               | 7.50     | 5                              | 7.6                         |
|                                      | "                                                                                                                                                                | 7.68     | 5                              | 8.2                         |
|                                      | "                                                                                                                                                                | 7.74     | 5                              | 2.4                         |
|                                      | "                                                                                                                                                                | 7.80     | 5                              | 2.0                         |
|                                      | "                                                                                                                                                                | 7.86     | 5                              | 2.8                         |
|                                      | 65                                                                                                                                                               | 7.60     | 5                              | 8.6                         |
|                                      | "                                                                                                                                                                | 7.72     | 5                              | 8.0                         |
|                                      | "                                                                                                                                                                | 7.80     | 5                              | 6.6                         |
|                                      | "                                                                                                                                                                | 7.93     | 5                              | 5.0                         |
|                                      | "                                                                                                                                                                | 8.04     | 5                              | 3.2                         |
|                                      | "                                                                                                                                                                | 8.27     | 5                              | 1.2                         |
|                                      | "                                                                                                                                                                | 8.35     | 5                              | 1.0                         |
|                                      | "                                                                                                                                                                | 7.53     | 10                             | 9.0                         |
|                                      | "                                                                                                                                                                | 7.75     | 10                             | 10.0                        |
|                                      | "                                                                                                                                                                | 7.97     | 10                             | 10.0                        |
|                                      | "                                                                                                                                                                | 8.15     | 10                             | 9.4                         |
|                                      | "                                                                                                                                                                | 8.30     | 10                             | 6.6                         |
|                                      | "                                                                                                                                                                | 8.48     | 10                             | 8.4                         |
|                                      | "                                                                                                                                                                | 8.65     | 10                             | 6.8                         |
|                                      | "                                                                                                                                                                | 8.72     | 10                             | 5.6                         |
|                                      | "                                                                                                                                                                | 8.92     | 10                             | 6.0                         |
|                                      | "                                                                                                                                                                | 9.10     | 10                             | 5.0                         |
|                                      | "                                                                                                                                                                | 9.25     | 10                             | 4.4                         |
|                                      | "                                                                                                                                                                | 8.65     | 20                             | 7.6                         |
|                                      | "                                                                                                                                                                | 8.90     | 20                             | 7.2                         |
|                                      | "                                                                                                                                                                | 9.10     | 20                             | 7.6                         |
|                                      | "                                                                                                                                                                | 9.30     | 20                             | 3.2                         |

TABLE 9

| ZINC RETAINED AS COMPARED TO TABLE 2 |                                                                                                                                                         |          |                                |                             |
|--------------------------------------|---------------------------------------------------------------------------------------------------------------------------------------------------------|----------|--------------------------------|-----------------------------|
| Conditions:                          | Initial Zinc = 10 ppm as Zn <sup>++</sup><br>T = 120° F.<br>Time = 24 hours<br>Treatment = AA/HPA, Mole Ratio AA:HPA = 3:1,<br>Molecular Weight = 6,000 | Water pH | Treatment Dosage (ppm actives) | Soluble Zinc Retained (ppm) |
|                                      | 7.27                                                                                                                                                    | 5        | 10                             |                             |
|                                      | 7.54                                                                                                                                                    | 5        | 10                             |                             |
|                                      | 7.77                                                                                                                                                    | 5        | 10                             |                             |
|                                      | 8.02                                                                                                                                                    | 5        | 8.4                            |                             |
|                                      | 8.08                                                                                                                                                    | 5        | 8.0                            |                             |

TABLE 11-continued

| ZINC RETAINED AS COMPARED TO TABLE 2 |                                                |                             |
|--------------------------------------|------------------------------------------------|-----------------------------|
| Conditions:                          | Initial Zinc = 10 ppm as $Zn^{++}$             |                             |
|                                      | T = 120° F.                                    |                             |
|                                      | Time = 24 hours                                |                             |
|                                      | Treatment = AA/HPA, Mole Ratio AA:HPA = 9.9:1. |                             |
|                                      | Molecular Weight = 6,000-10,000                |                             |
| Water pH                             | Treatment Dosage (ppm actives)                 | Soluble Zinc Retained (ppm) |
| 7.88                                 | 5                                              | 0.8                         |
| 8.20                                 | 5                                              | 0.6                         |
| 8.27                                 | 5                                              | 0.2                         |
| 8.58                                 | 5                                              | 0.2                         |
| 8.10                                 | 10                                             | 8.4                         |
| 8.13                                 | 10                                             | 8.4                         |
| 8.20                                 | 10                                             | 8.2                         |
| 8.25                                 | 10                                             | 8.6                         |
| 8.50                                 | 10                                             | 7.2                         |
| 8.74                                 | 10                                             | 6.0                         |
| 9.01                                 | 10                                             | 7.4                         |
| 9.14                                 | 10                                             | 7.6                         |
| 9.32                                 | 10                                             | 2.8                         |

TABLE 12

| ZINC RETAINED AS COMPARED TO TABLE 2 |                                                 |                             |
|--------------------------------------|-------------------------------------------------|-----------------------------|
| Conditions:                          | Initial Zinc = 10 ppm as $Zn^{++}$              |                             |
|                                      | T = 120° F.                                     |                             |
|                                      | Time = 24 hours                                 |                             |
|                                      | Treatment = AA/HPA, Mole Ratio AA:HPA = 19.8:1. |                             |
|                                      | Molecular Weight = 2,000-6,000                  |                             |
| Water pH                             | Treatment Dosage (ppm actives)                  | Soluble Zinc Retained (ppm) |
| 7.80                                 | 10                                              | 2.4                         |
| 7.83                                 | 10                                              | 2.4                         |
| 7.95                                 | 10                                              | 1.2                         |
| 8.08                                 | 10                                              | 1.0                         |
| 8.12                                 | 10                                              | 1.2                         |
| 8.25                                 | 10                                              | 1.2                         |
| 8.35                                 | 10                                              | 1.4                         |
| 8.15                                 | 20                                              | 4.6                         |
| 8.35                                 | 20                                              | 4.8                         |
| 8.52                                 | 20                                              | 5.2                         |
| 8.78                                 | 20                                              | 4.0                         |
| 8.62                                 | 30                                              | 8.4                         |
| 8.83                                 | 30                                              | 8.6                         |
| 8.88                                 | 30                                              | 8.2                         |
| 8.95                                 | 30                                              | 8.4                         |
| 9.02                                 | 30                                              | 7.4                         |
| 9.11                                 | 30                                              | 5.2                         |

TABLE 13

| ZINC RETAINED AS COMPARED TO TABLE 2 |                                    |                             |
|--------------------------------------|------------------------------------|-----------------------------|
| Conditions:                          | Initial Zinc = 10 ppm as $Zn^{++}$ |                             |
|                                      | T = 120° F.                        |                             |
|                                      | Time = 24 hours                    |                             |
|                                      | Treatment = AA/HPA,                |                             |
|                                      | Mole Ratio AA:HPA = 36:1,          |                             |
|                                      | Molecular Weight = 2,000-6,000     |                             |
| Water pH                             | Treatment Dosage (ppm actives)     | Soluble Zinc Retained (ppm) |
| 7.75                                 | 5                                  | 58                          |
| 7.79                                 | 5                                  | 2.6                         |
| 8.02                                 | 5                                  | 1.0                         |
| 8.34                                 | 5                                  | 0.2                         |
| 8.66                                 | 5                                  | 0.0                         |
| 8.27                                 | 10                                 | 7.0                         |
| 8.40                                 | 10                                 | 5.8                         |
| 8.50                                 | 10                                 | 7.6                         |
| 8.62                                 | 10                                 | 6.6                         |
| 8.87                                 | 10                                 | 6.6                         |
| 8.90                                 | 10                                 | 7.2                         |
| 9.03                                 | 10                                 | 7.8                         |
| 9.40                                 | 10                                 | 5.2                         |
| 8.79                                 | 20                                 | 9.0                         |
| 8.95                                 | 20                                 | 8.6                         |

TABLE 13-continued

| ZINC RETAINED AS COMPARED TO TABLE 2 |                                    |                             |
|--------------------------------------|------------------------------------|-----------------------------|
| Conditions:                          | Initial Zinc = 10 ppm as $Zn^{++}$ |                             |
|                                      | T = 120° F.                        |                             |
|                                      | Time = 24 hours                    |                             |
|                                      | Treatment = AA/HPA,                |                             |
|                                      | Mole Ratio AA:HPA = 36:1,          |                             |
|                                      | Molecular Weight = 2,000-6,000     |                             |
| Water pH                             | Treatment Dosage (ppm actives)     | Soluble Zinc Retained (ppm) |
| 9.05                                 | 20                                 | 8.6                         |
| 9.11                                 | 20                                 | 7.0                         |
| 9.21                                 | 20                                 | 7.8                         |
| 9.23                                 | 20                                 | 7.2                         |

15  
EFFICACY AS CORROSION INHIBITOR  
EXAMPLE 5

Having already demonstrated both the zinc precipitation problem related to zinc-containing corrosion inhibitor treatments in aqueous mediums and the resolution of this problem by combining the treatment with AA/HAA polymer, the following test results are presented to demonstrate, from a corrosion inhibition point of view, the benefits of the combined treatments.

The tests were each conducted with two non-pre-treated low carbon steel coupons which were immersed and rotated in aerated synthetic cooling water for a 3 or 4 day period. The water was adjusted to the desired pH and readjusted after one day if necessary; no further adjustments were made. Water temperature was 120° F. Rotational speed was maintained to give a water velocity of 1.3 feet per second past the coupons. The total volume of water was 17 liters. Cooling water was manufactured to give the following conditions:

|                       | SCW <sub>7</sub> (pH = 7) | SCW <sub>8</sub> (pH = 8) |
|-----------------------|---------------------------|---------------------------|
| 40 ppm Ca as $CaCO_3$ | 170                       | 170                       |
| ppm Mg as $CaCO_3$    | 110                       | 110                       |
| ppm $SiO_2$           | 15                        | 15                        |
| ppm $Na_2CO_3$        | 0                         | 100                       |

Corrosion rate measurement was determined by weight loss measurement. Prior to immersion, coupons were scrubbed with a mixture of trisodium phosphate-pumice, rinsed with water, rinsed with isopropyl alcohol and then air dried. Weight measurement to the nearest milligram was made. At the end of one day, a 45 weighed coupon was removed and cleaned. Cleaning consisted of immersion into a 50% solution of HCl for approximately 20 seconds, rinsing with tap water, scrubbing with a mixture of trisodium-pumice until clean, then rinsing with tap water and isopropyl alcohol. 50 When dry, a second weight measurement to the nearest milligram was made. At the termination of the tests, the remaining coupon was removed, cleaned and weighed.

55 Corrosion rates were computed by differential weight loss according to the following equation:

$$60 \text{ Corrosion Rate} = \frac{N^{\text{th}} \text{ Day Weight Loss} - 1^{\text{st}} \text{ Day Weight Loss}}{N - 1}$$

where N = 3 or 4.

65 The cooling water was prepared by first preparing the following stock solutions:

Solution A—212.4 g  $CaCl_2 \cdot 2H_2O/1$

Solution B—229.9 g  $MgSO_4 \cdot 7H_2O/1$

Solution C—25.5 g NaSiO<sub>3</sub>.9H<sub>2</sub>O/l  
Solution D—85 g Na<sub>2</sub>CO<sub>3</sub>/l

Treatment Solutions—1.7% solutions (1.7 g/100 ml)  
Then, these solutions were combined using the following order of addition:

1. To 17 l of de-ionized water add, with stirring, (a) 20 ml of Solution A, (b) 20 ml of Solution B and (c) 20 ml of Solution C.
2. Adjust pH to 6.
3. With stirring add treatment (except Zn<sup>2+</sup>).
4. Add o-PO<sub>4</sub> Solution (if used).
5. Adjust pH to 7.0 if necessary.
6. Add Zn<sup>2+</sup> Solution (if used).
7. (a) For SCW<sub>7</sub> adjust pH to 7.0, (b) For SCW<sub>8</sub> add 20 ml of Solution D and adjust pH to 8.0.

The results of these tests are reported below in Table 14 in terms of corrosion rates in mils per year (mpy).

TABLE 14

| CORROSION INHIBITION |        |                  |                         |                                 |    |                      |
|----------------------|--------|------------------|-------------------------|---------------------------------|----|----------------------|
| Polymer (ppm)        | AA:HPA | Molecular Weight | o-PO <sub>4</sub> (ppm) | Zinc (ppm as Zn <sup>2+</sup> ) | pH | Corrosion Rate (mpy) |
| 5                    | 3:1    | 6,000            | —                       | —                               | 7  | 155                  |
| 50                   | 3:1    | 6,000            | —                       | —                               | 7  | 35                   |
| —                    | —      | —                | 10                      | 2                               | 7  | 2.8                  |
| 5                    | 3:1    | 6,000            | 10                      | 2                               | 7  | 2.5                  |
| —                    | —      | —                | 5                       | 2                               | 7  | 8                    |
| 5                    | 3:1    | 6,000            | 5                       | 2                               | 7  | 3.0                  |
| 5                    | 1.8:1  | 6,000            | 10                      | 2                               | 7  | 2.1                  |
| None                 | —      | —                | —                       | —                               | 8  | 82                   |
| 30                   | 3:1    | 6,000            | —                       | —                               | 8  | 86                   |
| —                    | —      | —                | —                       | 10                              | 8  | 84                   |
| 5                    | 3:1    | 6,000            | —                       | 5                               | 8  | 13.6                 |
| 15                   | 3:1    | 6,000            | —                       | 10                              | 8  | 13.4                 |
| —                    | —      | —                | 5                       | 2                               | 8  | 21.5                 |
| 5                    | 3:1    | 6,000            | 5                       | 2                               | 8  | 1.5                  |
| 5                    | 1.8:1  | 6,000            | 5                       | 2                               | 8  | 0                    |
| —                    | —      | —                | 3                       | 2                               | 8  | 76                   |
| 5                    | 3:1    | 6,000            | 3                       | 2                               | 8  | 1.6                  |
| 5                    | 1.8:1  | 6,000            | 3                       | 2                               | 8  | 8.6                  |

While the comparative test results were not so pronounced at pH=7, the comparative results at pH=8 were considered to be rather dramatic. Even though the AA/HPA polymer alone demonstrated little, if any, efficacy as a corrosion inhibitor, when combined with the zinc-containing treatments, the combined treatments demonstrated significantly enhanced results as corrosion inhibitors. For example, at pH=8, the corrosion inhibition efficacy of 30 ppm active polymer alone (86 mpy) and 10 ppm Zn<sup>2+</sup> alone (84 mpy) appeared to be non-existent as compared to the untreated system (82 mpy); however, when only 5 ppm polymer were combined with only 5 ppm Zn<sup>2+</sup>, the corrosion rate decreased to 13.6 mpy.

## EXAMPLE 6

Additional tests were conducted to demonstrate the efficacy of AA/HPA copolymer in combination with a cooling water treatment containing zinc, orthophosphate and water-soluble chromate. This cooling water treatment is taught in U.S. Pat. No. 2,900,222 to Kahler et al. The copolymer was also tested in combination with zinc and water-soluble chromate, the latter two components individually being well-known cooling water treatment compounds.

The test procedures were generally the same as those described in Example 5; spinner tests were used, and coupon weight loss measurements provided the basis

for calculating corrosion rates. Test conditions were as follows:

|   |                                    |   |           |
|---|------------------------------------|---|-----------|
| 5 | spinner volume                     | = | 17 liters |
|   | ppm calcium as CaCO <sub>3</sub>   | = | 170       |
|   | ppm magnesium as CaCO <sub>3</sub> | = | 110       |
|   | ppm chloride                       | = | 121       |
|   | ppm sulfate                        | = | 106       |
|   | ppm silica                         | = | 15        |
|   | M-alkalinity                       | = | 80 ppm    |
|   | bulk water temperature             | = | 120° F.   |
|   | pH                                 | = | 8.0       |

The results of these tests are reported below in Table 15 in terms of corrosion rates in mils per year (mpy). The copolymer had a mole ratio of AA:HPA of 3:1 and a molecular weight of 6,000. The chromate used was sodium dichromate, Na<sub>2</sub>Cr<sub>2</sub>O<sub>7</sub>.2H<sub>2</sub>O.

TABLE 15

| 20 | Copolymer (ppm) | CORROSION INHIBITOR     |            |                | Corrosion Rate <sup>1</sup> |
|----|-----------------|-------------------------|------------|----------------|-----------------------------|
|    |                 | o-PO <sub>4</sub> (ppm) | Zinc (ppm) | Chromate (ppm) |                             |
| 25 | 16              | —                       | —          | —              | 25 <sup>2</sup>             |
|    | 5               | 5                       | 5          | 1              | 0.44                        |
|    | 17              | —                       | —          | —              | 33                          |
|    | 5               | 5                       | 5          | 2              | 0.56                        |
|    | 22              | —                       | —          | —              | 44                          |
|    | 10              | 9.2                     | 9.2        | 3.6            | 0.66                        |
|    | 20              | 5                       | 5          | 2              | 0                           |
| 30 | 6.67            | 6.67                    | 6.67       | —              | 39                          |
|    | 5               | 5                       | 5          | —              | 0                           |
|    | —               | 8.33                    | 8.33       | 8.33           | 0.44                        |
|    | 5               | —                       | 5          | 5              | 0                           |
|    | 5               | —                       | 5          | 2              | 0.25                        |

<sup>1</sup>Unless indicated otherwise, these values each represent an average for 3 runs.

<sup>2</sup>Average for 2 runs.

As can be seen from the results of Table 15, the AA/HPA in combination with zinc/chromate and zinc/chromate/orthophosphate proved to be efficacious for corrosion inhibition.

Having thus described the invention what is claimed is:

1. A method for reducing the amount of corrosion of metal surfaces in contact with an aqueous medium prone to zinc precipitation comprising adding to said aqueous medium an effective amount for the purpose of effectiveness:

- (i) water-soluble zinc compound,
- (ii) water-soluble chromate compound, and
- (iii) water-soluble polymer comprising moieties derived from acrylic acid or water-soluble salt thereof and moieties of hydroxylated lower alkyl acrylate, wherein the moieties of said polymer have the following formulas:



wherein R is hydrogen or a lower alkyl of from 1 to 3 carbon atoms; R<sub>1</sub> is OH, NH<sub>2</sub> or OM where M is a water-soluble cation; R<sub>2</sub> is a lower alkyl of from

about 2 to 6 carbon atoms, R<sub>3</sub> is H or lower alkyl of from 1 to 3 carbon atoms and the mole ratio of x:y is 1:4 to 36:1, said polymer being capable of retaining a corrosion inhibiting amount of said zinc compound in soluble form in said aqueous medium.

2. A method according to claim 1, wherein said zinc compound is added in an amount sufficient to provide from about 0.5 to about 25 parts of zinc ion per million parts of aqueous medium, said polymer is added in an amount of from about 0.5 to about 200 parts of polymer per million parts of aqueous medium, and said chromate compound is added in an amount of from about 1 to about 150 parts of chromate compound per million parts of aqueous medium.

3. A method according to claim 2, wherein said zinc compound is added in an amount sufficient to provide from about 2 to about 10 parts of zinc ion per million parts of aqueous medium, said polymer is added in an amount of from about 2 to about 50 parts of polymer per million parts of aqueous medium, and said chromate compound is added in an amount of about 1 to about 50 parts per million.

4. A method according to claim 3, wherein said mole ratio of z:y is 1:1 to 11:1.

5. A method according to claim 4, wherein said polymer has a molecular weight of from about 1,000 to about 50,000.

6. A method according to claim 5, wherein said polymer has a molecular weight of from about 2,000 to about 6,000.

7. A method according to claim 6, wherein said mole ratio of z:y is 1:1 to 5:1.

8. A method according to claim 7, wherein said polymer has a molecular weight of from about 2,000 to about 6,000.

9. A method according to claim 5 or 8, wherein said aqueous medium is cooling water.

10. A method according to claim 9 wherein said polymer is a copolymer of acrylic acid or water soluble salt thereof and 2-hydroxypropyl acrylate.

11. A method according to claim 10 wherein said aqueous medium has a pH of from about 6.5 to about 9.5.

12. A method for reducing the amount of corrosion of metal surfaces in contact with an aqueous medium prone to zinc precipitation comprising adding to said aqueous medium an effective amount for the purpose of effective:

- (i) water-soluble zinc compound,
- (ii) water-soluble orthophosphate or precursor thereof,
- (iii) water-soluble chromate compound, and
- (iv) water-soluble polymer comprising moieties derived from acrylic acid or water-soluble salt thereof and moieties of hydroxylated lower alkyl acrylate, wherein the moieties of the polymer have the following formulas:



wherein R is hydrogen or a lower alkyl of from 1 to 3 carbon atoms; R<sub>1</sub> is OH, NH<sub>2</sub> or OM where M is a water-soluble cation; R<sub>2</sub> is a lower alkyl of from about 2 to 6 carbon atoms, R<sub>3</sub> is H or lower alkyl of from 1 to 3 carbon atoms and the mole ratio of x:y is 1:4 to 36:1, said polymer being capable of retaining a corrosion inhibiting amount of said zinc compound in soluble form in said aqueous medium.

13. A method according to claim 12, wherein said zinc compound is added in an amount sufficient to provide from about 0.5 to about 25 parts of zinc ion per million parts of aqueous medium, said polymer is added in an amount of from about 0.5 to about 200 parts of polymer per million parts of aqueous medium, said orthophosphate or precursor thereof is added in an amount of from about 1 to about 200 parts per million, and said chromate compound is added in an amount of from about 1 to about 150 parts per million.

14. A method according to claim 13, wherein said zinc compound is added in an amount sufficient to provide from about 2 to about 10 parts of zinc ion per million parts of aqueous medium, said polymer is added in an amount of from about 2 to about 50 parts of polymer per million parts of aqueous medium, said orthophosphate or precursor thereof is added in an amount of from about 2 to about 50 parts per million, and said chromate compound is added in an amount of from about 1 to about 50 parts per million.

15. A method according to claim 14, wherein said mole ratio of x:y is 1:1 to 11:1.

16. A method according to claim 15, wherein said polymer has a molecular weight of from about 1,000 to about 50,000.

17. A method according to claim 16, wherein said polymer has a molecular weight of from about 2,000 to about 6,000.

18. A method according to claim 17, wherein said mole ratio of x:y is 1:1 to 5:1.

19. A method according to claim 16 or 18, wherein said aqueous medium is cooling water.

20. A method according to claim 19, wherein said polymer is a copolymer of acrylic acid or water-soluble salt thereof and 2-hydroxypropyl acrylate.

21. A method according to claim 19, wherein said aqueous medium has a pH of from about 6.5 to about 9.5.

22. A method in accordance with claim 12 wherein said water soluble orthophosphate or precursor thereof comprises a member selected from the group consisting of aminotrimethylene phosphonic acid, hydroxyethylidene diphosphonic acid and water soluble salts thereof.

23. A method in accordance with claim 22 wherein said water soluble orthophosphate or precursor thereof comprises hydroxyethylidene diphosphonic acid and water soluble salt forms thereof.

\* \* \* \* \*